

[72] Inventors Shiro Kimura;  
Yoshiyuki Nakazawa; Yasuharu  
Nakamura; Akira Sato; Masao Sawahara;  
Katsuji Yoshida, all of Kanagawa, Japan

[21] Appl. No. 842,361

[22] Filed July 16, 1969

[45] Patented Nov. 9, 1971

[73] Assignee Fuji Photo Film Co., Ltd.  
Kanagawa, Japan

[32] Priority July 16, 1968

[33] Japan

[31] 43/50099

[54] **OPTICALLY SENSITIZED SILVER HALIDE  
PHOTOGRAPHIC EMULSIONS**  
4 Claims, No Drawings

[52] U.S. Cl. 96/132,  
96/99

[51] Int. Cl. G03c 1/10  
[50] Field of Search. 96/106

[56] References Cited

UNITED STATES PATENTS

|           |        |                 |       |        |
|-----------|--------|-----------------|-------|--------|
| 3,255,012 | 6/1966 | Glockner et al. | ..... | 96/106 |
| 3,369,902 | 2/1968 | Abbott          | ..... | 96/106 |

Primary Examiner—Norman G. Torchin

Assistant Examiner—John L. Goodrow

Attorney—Sughrue, Rothwell, Mion, Zinn and Macpeak

**ABSTRACT:** A photographic silver halide emulsion containing a sensitizing dye represented by the formula:



wherein Z represents a member from the group consisting of a sulfur atom or a selenium atom; A represents a member from the group consisting of a hydrogen atom, a lower alkyl group or a hydroxyl group; B represents a member from the group consisting of a hydrogen atom or a lower alkyl group; R and R' represent a member from the group consisting of a lower alkyl group or a substituted alkyl group, and at least one of R and R' represent a member from the group consisting of a sulfoalkyl group or a carboxyalkyl group; X represents an anion; and n represents 0 or 1, n being 0 when the sensitizing dye is an intramolecular salt.

A photographic light-sensitive element comprising the above emulsion on a support is also claimed.

OPTICALLY SENSITIZED SILVER HALIDE  
PHOTOGRAPHIC EMULSIONS

BACKGROUND OF THE INVENTION

1. Field of the Invention

The present invention relates to a silver halide photographic emulsion containing a sensitizing dye, and more particularly to a silver halide photographic emulsion containing a thia-2'-cyanin sensitizing dye or a seleno-2'-cyanin sensitizing dye which has a hydroxyl group in the 5-position of the benzothiazole nucleus or the benzoselenazole nucleus, and in which a nucleus nitrogen atom in either of the heterocyclic rings is substituted by a sulfoalkyl group or carboxyalkyl group.

2. Description of the Prior Art

The spectral sensitizing technique of adding certain sensitizing dyes to a silver halide emulsion to further enlarge its light sensitive wavelength range has been well known in the manufacturing technique of silver halide photographic emulsion. Also, the sensitizing dye to be contained in the silver halide photographic emulsion should be such as to provide the desired spectral sensitivity without having a bad influence upon the photographic sensitive materials.

However, a silver halide photographic emulsion which is spectrally sensitized often brings about a color-stain caused by the sensitizing dye after the conventional treatments of development, fixing, washing with water, etc. In black and white photography, the color-stain derived from this dye will act to impede visible judgment of the image during printing by virtue of short wavelength light or platemaking.

Further, there will also occur other problems, as it is unfeasible to obtain a print having an excellent whiteness (one aspect), one cannot obtain the intended color reproduced image in case of color photography. The present invention, as explained hereafter, overcomes these faults.

SUMMARY OF THE INVENTION

The present invention, in essence, provides a silver halide emulsion containing a sensitizing dye represented by the formula:



wherein Z represents a member from the group consisting of a sulfur atom or a selenium atom; A represents a member from the group consisting of a hydrogen atom, a lower alkyl group or a hydroxyl group; B represents a member from the group consisting of a hydrogen atom or a lower alkyl group; R and R' represent a member from the group consisting of a lower alkyl group or a substituted alkyl group, and at least one of R and R' represent a member from the group consisting of a sulfoalkyl group or a carboxyalkyl group; X represents an anion; and n represents 0 or 1, n being 0 when the sensitizing dye is an intramolecular salt.

The above emulsion finds particular use in a photographic light-sensitive element, wherein the emulsion is carried on a support.

Therefore, an object of the present invention is to provide a silver halide photographic emulsion having lower color-stain caused by the sensitizing dye, which is produced after carrying out the conventional treatments of development, fixing, washing with water, etc. Further, the emulsion will have a high sensitivity in the green sensitive range.

Another object of the present invention is to provide a silver halide photographic emulsion having a high sensitivity in the green sensitive range used for a printing or duplication

orthofilm, cinema recording film, and indirect photography Roentgen film for medical treatment, etc.

The above objects of the present invention have been accomplished by incorporating at least one 5-hydroxythia-2'-cyanin or 5-hydroxyseleno-2'-cyanin sensitizing dyes represented by the formula



10  
15

wherein Z represents a sulfur atom or a selenium atom; A represents a hydrogen atom, a lower alkyl group, i.e., one-four carbon atoms, (for example, methyl group, ethyl group, etc.), or a hydroxyl group; B represents a hydrogen atom, or a lower alkyl group, i.e., one-four carbon atoms, (for example, methyl group, ethyl group, etc.); R and R' represent an alkyl group (for example, methyl group, ethyl group, propyl group, etc.) or a substituted alkyl group (for example, carboxymethyl group, β-carboxy-ethyl group, α-carboxypropyl group, α-carboxy-butyl group, β-hydroxyethyl group, β-acetoxyethyl group, ethoxycarbonylmethyl group, β-ethoxycarbonyl-ethyl group, β-sulfoethyl group, α-sulfopropyl group, α-sulfonybutyl group, δ-sulfonybutyl group, benzyl group, phenethyl group, carboxybenzyl group, vinyl methyl group (=alkyl group), etc.) and at least one of R and R' represents a sulfoalkyl group of one-five carbon atoms or a carboxyalkyl group of one-five carbon atoms; X<sup>1</sup> represents an anion; and n is 0 or 1, and when the dye is an intramolecular salt in a silver halide photographic emulsion, n is 0.

20  
25  
30  
35

To further define components R and R', the term "alkyl group" means an alkyl group having from one to four carbon atoms. However, the sulfosubstituted alkyl group can have from one to six carbon atoms and the carboxy substituted alkyl group can have from one to 10 carbon atoms. Further, acceptable substituents on the alkyl group which may be component R or R' are carboxyl groups, hydroxyl groups, alkoxy groups, a sulfogroup, an aralkyl group or a vinyl group.

40  
45

As heretofore indicated X<sup>1</sup> represents an anion, such as a halogen ion (Cl, Br, I), a p-toluenesulfonate ion, -C<sub>6</sub>H<sub>4</sub>-O-SO<sub>3</sub><sup>1</sup>, etc.

The sensitizing dye represented by the above formula can be synthesized by conventional processes, that is, it can be obtained by condensing a heterocyclic quaternary ammonium salt represented by the formula:



55  
60  
65

wherein D represents a hydrogen atom, a lower alkyl group of one-four carbon atoms (for example, methyl group, ethyl group, etc.), or an alkoxy group of one-four carbon atoms (for example, methoxy group, ethoxy group, etc.); R, X, and n have the same meaning as in formula (I), and R'' represents a methyl group, an ethyl group, or a phenyl group, etc., and a heterocyclic quaternary ammonium salt represented by the formula



70  
75

75

wherein Z, B, R', X, and n have the same meaning -position in formula (I), in the presence of an organic base (for example, triethylamine) in ethanol or pyridine. A 5-hydroxy benzothiazole, 5-hydroxy-6-alkyl (methyl or ethyl) benzothiazole, or 5-hydroxy benzoselenazole, 5-hydroxy-6-alkyl (methyl or ethyl) benzoselenazole which is starting material for the compound represented by the formula (III) can be synthesized by the hydrolysis of 5-alkoxy (methoxy or ethoxy) benzothiazole, 5-alkoxy-6-alkyl (methyl or ethyl) benzothiazole, 5-alkoxy (methoxy or ethoxy) 10 benzoselenazole, or 5-alkoxy-6-alkyl (methyl or ethyl) benzoselenazole with a mineral acid, for example hydrobromic acid. Also the sensitizing dye represented by formula (I) can be obtained by the hydrolysis of a sensitizing dye having an alkoxy group in the 5-position of the benzothiazole nucleus, or of a benzoselenazole nucleus with a mineral acid.

Further, the sensitizing dye of formula (I) used in the present invention as A is a hydroxyl group, may be obtained by the hydrolysis of a sensitizing dye of formula (I) wherein group A is replaced with an alkoxy group, or wherein group A is replaced with an alkoxy group and the 5-position of the benzothiazole nucleus or the benzoselenazole nucleus has an alkoxy group, with a mineral acid.

Examples of preparing the sensitizing dye used in the present invention will be described, and further sensitizing 25 dyes used in the present invention will be listed herein. However, the present invention is not limited by these dyes.

#### Intermediate (1)

3-ethyl-5-hydroxy-2-methylbenzothiazolium p-toluenesulfonate 30



10 g. of 5-hydroxy-2-methylbenzothiazole and 18 g. of ethyl p-toluenesulfonate were melted by heating at 160° C. and reacted for 4 hours. The resulting crystal, after washing, was recrystallized from a mixed solvent of methanol and isopropanol to obtain intermediate (1), melting at 182° C. Yield 19 g.

#### Intermediate (2)

Anhydro 5-hydroxy-2-methyl-3-( $\delta$ -sulfonylbutyl)benzothiazolium hydroxide 50



5 g. of 5-hydroxy-2-methylbenzothiazole and 4 g. of butane sulfone were melted by heating at 160° C. and reacted for 1

hour. The resulting crystal was washed with acetone to provide 6 g. of intermediate (2) melting at 278° C.

#### Dye (7)

Anhydro 1'-ethyl-5-hydroxy-6'-methyl-3-( $\delta$ -sulfonylbutyl)-thia-2'-cyanin hydroxide



1.2 g. of 1-ethyl-2-ethylmercapto-6-methyl-quinolinium-p-toluenesulfonate and 1 g. of anhydro-5-hydroxy-2-methyl-3-( $\delta$ -sulfonylbutyl)benzothiazolium hydroxide were reacted for 2 hours while refluxing at 78° C. in 100 cc. of ethanol and 6 cc. of triethylamine. The precipitated crystal was separated by filtration and was recrystallized from a solvent mixture of methanol and chloroform to obtain 12 g. of dye (7) melting at above 300° C.

#### Dye (18)

Anhydro 5,6'-dihydroxy-1'-ethyl-3-( $\delta$ -sulfonylpropyl)-thia-2'-cyanin hydroxide



1 g. of anhydro 1'-ethyl-5-hydroxy-6'-methoxy-3-( $\delta$ -sulfonylpropyl)-thia-2'-cyanin hydroxide was reacted for 7 hours while refluxing at 100° C. in 30 ml. of 47 percent hydrobromic acid. After cooling, 500 ml. of water was added thereto and the precipitated dye was separated by filtration, washed well, and then recrystallized from a solvent mixture of methanol, chloroform and triethylamine to obtain 600 mg. of dye (18) melting at above 300° C.

55



Other sensitizing dyes used in the present invention may be prepared in a similar manner to the aforesaid procedure, and typical dyes are illustrated in the following table, together with the above-prepared dyes.

| No. of dye | Z              | A               | B | R                                                             | R'                                                            | X | M.P.,<br>°C. | MeOH<br>λ <sub>max.</sub> ,<br>μμ |
|------------|----------------|-----------------|---|---------------------------------------------------------------|---------------------------------------------------------------|---|--------------|-----------------------------------|
| 1          | S              | H               | H | —C <sub>2</sub> H <sub>5</sub>                                | —(CH <sub>2</sub> ) <sub>3</sub> SO <sub>3</sub> <sup>-</sup> |   | 300          | 496                               |
| 2          | S              | H               | H | —(CH <sub>2</sub> ) <sub>3</sub> SO <sub>3</sub> <sup>-</sup> | —C <sub>2</sub> H <sub>5</sub>                                |   | 300          | 497.5                             |
| 3          | S <sup>+</sup> | H               | H | —C <sub>2</sub> H <sub>5</sub>                                | —(CH <sub>2</sub> ) <sub>3</sub> SO <sub>3</sub> <sup>-</sup> |   | 300          | 503                               |
| 4          | S <sup>+</sup> | H               | H | —(CH <sub>2</sub> ) <sub>3</sub> SO <sub>3</sub> <sup>-</sup> | —(CH <sub>2</sub> ) <sub>3</sub> SO <sub>3</sub> <sup>-</sup> |   | 300          | 505                               |
| 5          | S              | CH <sub>3</sub> | H | —C <sub>2</sub> H <sub>5</sub>                                | —(CH <sub>2</sub> ) <sub>3</sub> SO <sub>3</sub> <sup>-</sup> |   | 300          | 501                               |
| 6          | S              | CH <sub>3</sub> | H | —C <sub>2</sub> H <sub>5</sub>                                | —(CH <sub>2</sub> ) <sub>3</sub> SO <sub>3</sub> <sup>-</sup> |   | 300          | 502                               |
| 7          | S              | CH <sub>3</sub> | H | —C <sub>2</sub> H <sub>5</sub>                                | —(CH <sub>2</sub> ) <sub>3</sub> SO <sub>3</sub> <sup>-</sup> |   | 300          | 502                               |
| 8          | S              | CH <sub>3</sub> | H | —CH <sub>3</sub>                                              | —(CH <sub>2</sub> ) <sub>3</sub> SO <sub>3</sub> <sup>-</sup> |   | 300          | 500                               |
| 9          | S              | CH <sub>3</sub> | H | —CH <sub>3</sub>                                              | —(CH <sub>2</sub> ) <sub>3</sub> SO <sub>3</sub> <sup>-</sup> |   | 300          | 500                               |
| 10         | S              | CH <sub>3</sub> | H | —(CH <sub>2</sub> ) <sub>3</sub> SO <sub>3</sub> <sup>-</sup> | —C <sub>2</sub> H <sub>5</sub>                                |   | 300          | 503                               |
| 11         | S              | CH <sub>3</sub> | H | —(CH <sub>2</sub> ) <sub>3</sub> CONO                         | —(CH <sub>2</sub> ) <sub>3</sub> SO <sub>3</sub> <sup>-</sup> |   | 300          | 500                               |

Continued.

| No. of dye | Z  | A               | B               | R                                                             | R'                                                                                               | X   | M.P.,<br>°C. | MeOH.<br>λ <sub>max.</sub><br>μ |
|------------|----|-----------------|-----------------|---------------------------------------------------------------|--------------------------------------------------------------------------------------------------|-----|--------------|---------------------------------|
| 12         | S  | CH <sub>3</sub> | H               | -(CH <sub>2</sub> ) <sub>3</sub> SO <sub>3</sub> <sup>-</sup> | -(CH <sub>2</sub> ) <sub>3</sub> SO <sub>3</sub> HN(C <sub>2</sub> H <sub>5</sub> ) <sub>3</sub> | 297 | 505          |                                 |
| 13         | S  | CH <sub>3</sub> | H               | -C <sub>2</sub> H <sub>5</sub>                                | -CH <sub>2</sub> CH <sub>2</sub> COO <sup>-</sup>                                                | 218 | 502          |                                 |
| 14         | Se | CH <sub>3</sub> | H               | -C <sub>2</sub> H <sub>5</sub>                                | -(CH <sub>2</sub> ) <sub>3</sub> SO <sub>3</sub> <sup>-</sup>                                    | 300 | 507.5        |                                 |
| 15         | Se | CH <sub>3</sub> | H               | -(CH <sub>2</sub> ) <sub>3</sub> SO <sub>3</sub> <sup>-</sup> | -(CH <sub>2</sub> ) <sub>3</sub> SO <sub>3</sub> HN(Et) <sub>3</sub>                             | 288 | 512.5        |                                 |
| 16         | S  | CH <sub>3</sub> | CH <sub>3</sub> | -C <sub>2</sub> H <sub>5</sub>                                | -(CH <sub>2</sub> ) <sub>3</sub> SO <sub>3</sub> <sup>-</sup>                                    | 300 | 506          |                                 |
| 17         | S  | CH <sub>3</sub> | H               | -C <sub>2</sub> H <sub>5</sub>                                | -CH <sub>2</sub> COO <sup>-</sup>                                                                | 259 | 503          |                                 |
| 18         | S  | OH              | H               | -C <sub>2</sub> H <sub>5</sub>                                | (C <sub>2</sub> H <sub>5</sub> ) <sub>3</sub> SO <sub>3</sub> <sup>-</sup>                       | 300 | 510          |                                 |
| 19         | Se | OH              | H               | -C <sub>2</sub> H <sub>5</sub>                                | (CH <sub>2</sub> ) <sub>3</sub> SO <sub>3</sub> <sup>-</sup>                                     | 300 | 516          |                                 |

The sensitizing dye used in the present invention can spectrally sensitize a silver halide photographic emulsion, in particular, is effective for enlarging the spectrally sensitive range of gelatino silver halide photographic emulsion, and also can satisfactorily sensitize a photographic emulsion containing other hydrophilic colloids than gelatin, for example, agar agar, water-soluble cellulose derivatives, polyvinyl alcohol, and other synthetic and natural hydrophilic resins.

The silver halide to be used in the emulsion of the present invention can be various silver salts such as silver chloride, silver bromide, silver iodobromide, silver chlorobromide, and silver chloroiodobromide.

The sensitized photographic emulsion of the present invention may be prepared by adding one or more kinds of sensitizing dye to the photographic emulsion by the conventional method. Most practically, a solution of the dye dissolved in a suitable solvent, such as methanol, ethanol, etc. is added to the emulsion.

The amount of sensitizing dye to be added to the emulsion can be varied over the broad range of 5 to 150 mg. per 1 kg. of emulsion, according to the desired final objects.

The photographic emulsion of the present invention can be hypersensitized, and supersensitized. In the preparation of the photographic emulsion of the present invention, additives conventionally used, such as, a sensitizer, a stabilizer, a toning agent, a hardening agent, a surface active agent, an antifogging agent, a plasticizer, a developing promotor, a coupler, and a fluorescent whitening agent, may further be added to the emulsion by any conventional method.

The photographic emulsion can be applied to a suitable support, such as a glass, a film of cellulose derivative, a film of synthetic resin, or a baryta paper by any conventional method.

By way of example, the invention will now be defined with greater specificity.

The sensitizing dye of the present invention, as shown above, was added to silver iodobromide emulsion (AgI:AgBr=7 moles: 93 moles) to prepare a photographic emulsion. The emulsion was coated on a film base of cellulose triacetate and, after drying, exposed to a "day light" of 64 lux (corresponding to 5400° K) through a Fuji No. 17 filter (a green filter, transparent maximum at 525 to 530 μ, manufactured by Fuji Photographic Film Co., Ltd.) and developed.

The developing solution of the composition shown in table 1 was employed at 20° C. for the development temperature.

TABLE 1

|                                |            |
|--------------------------------|------------|
| N-methyl-p-aminophenol sulfate | 20 g.      |
| Hydroquinone                   | 5.0 g.     |
| Cadmium sulfate                | 100 g.     |
| Borax                          | 2.0 g.     |
| Water                          | To 1 liter |

Table 2 shows the spectral sensitivity and the sensitizing maximum, and table 3 shows the sensitivity and the color-stain concentration of typical sensitizing dyes of the present invention, in comparison with those of other dyes. As is apparent from table 3, the sensitizing dyes used in the present invention are superior to sensitizing dyes 20, 21, 22 and 23, which have the structures shown below, (these dyes are known as green sensitive sensitizing dyes) in sensitivity and in color-stain density.

TABLE 2

| 15 | Sensitizing | Mg. mole/kg.<br>emulsion | Emulsion | Sensitizing<br>max. (mμ) | Sensitivity |
|----|-------------|--------------------------|----------|--------------------------|-------------|
| 1  | ...         | 0.08                     | AgBr/1   | 555-560                  | 3,660       |
| 2  | ...         | 0.08                     | AgBr/1   | 555-560                  | 4,000       |
| 3  | ...         | 0.08                     | AgBr/1   | 565-570                  | 3,840       |
| 4  | ...         | 0.08                     | AgBr/1   | 570                      | 3,280       |
| 5  | ...         | 0.08                     | AgBr/1   | 550                      | 4,000       |
| 6  | ...         | 0.08                     | AgBr/1   | 565                      | 3,300       |
| 7  | ...         | 0.08                     | AgBr/1   | 555                      | 3,640       |
| 8  | ...         | 0.08                     | AgBr/1   | 560                      | 3,640       |
| 9  | ...         | 0.08                     | AgBr/1   | 550                      | 3,500       |
| 10 | ...         | 0.08                     | AgBr/1   | 555                      | 3,500       |
| 11 | ...         | 0.08                     | AgBr/1   | 552-560                  | 3,780       |
| 12 | ...         | 0.08                     | AgBr/1   | 550-555                  | 3,300       |
| 13 | ...         | 0.08                     | AgBr/1   | 558                      | 5,180       |
| 14 | ...         | 0.08                     | AgBr/1   | 560                      | 2,800       |
| 15 | ...         | 0.08                     | AgBr/1   | 565                      | 3,000       |
| 16 | ...         | 0.08                     | AgBr/1   | 560                      | 4,550       |
| 17 | ...         | 0.08                     | AgBr/1   | 550                      | 4,800       |
| 18 | ...         | 0.08                     | AgBr/1   | 562                      | 3,600       |
| 19 | ...         | 0.08                     | AgBr/1   | 570-580                  | 2,100       |

The value of the sensitivity shows the value on exposing a silver iodobromide emulsion to a light through a Fuji No. 17 filter as 100 for the green sensitivity of the emulsion not containing a dye.

35

TABLE 3

| 40 | Sensitizing dye | Mg. mole/kg.<br>emulsion | Emulsion | Sensitivity | Density of<br>color-stain |
|----|-----------------|--------------------------|----------|-------------|---------------------------|
| 3  | ...             | 0.08                     | AgBr/1   | 3,840       | 0.08                      |
| 10 | ...             | 0.08                     | AgBr/1   | 3,500       | 0.08                      |
| 15 | ...             | 0.08                     | AgBr/1   | 3,000       | 0.08                      |
| 17 | ...             | 0.08                     | AgBr/1   | 4,800       | 0.09                      |
| 20 | ...             | 0.08                     | AgBr/1   | 3,100       | 0.15                      |
| 21 | ...             | 0.08                     | AgBr/1   | 3,100       | 0.15                      |
| 22 | ...             | 0.08                     | AgBr/1   | 2,200       | 0.15                      |
| 23 | ...             | 0.08                     | AgBr/1   | 2,500       | 0.15                      |
| 24 | ...             | 0.08                     | AgBr/1   | 3,000       | 0.20                      |

<sup>1</sup> Control coloring matter.

The color-stain value shows the density through a Fuji No. 17 filter (transparent maximum 525 to 530 mμ, manufactured by Fuji Photographic Film Co., Ltd.)

## CONTROL DYE FORMULAS





As a final point, for instance, in intermediate (I), the p-toluene sulfonate ion



is bonded with the cation, that is



Accordingly, the "bondings" will be clear to one skilled in the art. For instance, in the general  $(X^1)^n$  does not represent a floating bond, but generally represents an anion. The anion is bonded with the cation, that is



What is claimed is:

1. A photographic silver halide emulsion containing a sensitizing dye represented by the formula

5

10

15



wherein Z represents a member from the group consisting of a sulfur atom or a selenium atom; A represents a member from the group consisting of a hydrogen atom, a lower alkyl group or a hydroxyl group; B represents a member from the group consisting of a hydrogen atom or a lower alkyl group; R and R' represent a member from the group consisting of a lower alkyl group or a substituted alkyl group, and at least one of R and R' represent a member from the group consisting of a sulfoalkyl group or a carboxyalkyl group; X represents an anion; and n represents 0 or 1, n being 0 when the sensitizing dye is an intramolecular salt.

2. The silver halide photographic emulsion as set forth in claim 1, wherein the sensitizing dye is a thia-2'-cyanin compound.

3. The silver halide photographic emulsion as set forth in claim 1, wherein the sensitizing dye is a selena-2'-cyanin compound.

35 4. A photographic light-sensitive element comprising a support having thereon the photographic silver halide emulsion layer as set forth in claim 1.

40

45

50

55

60

65

70

75